

## UNITED STATES PATENT OFFICE

2,607,676

## HARD METAL COMPOSITIONS

Jacob Kurtz, Teaneck, N. J.

No Drawing. Application June 1, 1949,  
Serial No. 96,615

9 Claims. (Cl. 75—136)

1

This invention relates to hard metal compositions, especially to hard metal compositions suitable for hot pressing in combination with non metallic abrasive grains, such as diamonds, or hard metallic abrasive and cutting grains, and/or pieces, such as cemented hard carbides, having extensive adaptations in the mining and oil well industries.

It is an object of this invention to provide a material composition to be used as matrix, that is hard, tough, abrasion resistant, easy to form and press, that is easily welded to itself, and to any suitable shank material, commonly used to attach the diamond impregnated unit or the like to a power driven shaft.

It is a further object of this invention to provide a new composition of material particularly adapted to be used in combination with inserted tungsten carbide tips in rotary type rock drilling bits. Heretofore making diamond drill bits and the like was a long tedious process. The desired quality of hardness and toughness of the matrix material was difficult to achieve and control, and the crown containing the diamonds required an additional soldering or brazing operation to bond it to the steel shank. Frequently, due to marked differences in the expansion coefficients between the crown and the shank, the crown cracked and broke away from the shank, or strains would be set up in the structure to cause the crown to break away shortly after it was put into service. Likewise when using cemented carbide inserts, the inserts would crack away from the main body of the material. The main body of the material would soon wear away, or if made sufficiently hard would crack in service shortly thereafter.

Heretofore the hard cemented carbide inserts would have to be brazed into the holder as a separate operation, and due to the marked differences of expansion between the shank and the carbide inserts, thermal strains would develop to cause cracking away of the cemented carbide at the time of making the braze or shortly after putting the unit to work.

The hard matrix material of the present invention and the method of producing it entirely eliminates the aforementioned difficulties. Briefly described, the hard alloy of the present invention consists essentially of refractory metal carbides, tungsten carbide for example, cobalt, nickel, manganese, copper, and a small but effective amount of beryllium combined in the proportions and according to the method described herebelow:

I first provide a refractory tungsten carbide,

2

200 mesh or finer made by any known means. Instead of tungsten carbide, I may use any of the refractory metal carbides, titanium, zirconium, vanadium, chromium, tantalum and molybdenum or suitable combinations of carbides from this group—for example a mixture of 85% tungsten carbide and 15% titanium carbide. A mixture of 50% tungsten carbide, 35% molybdenum carbide, 15% titanium carbide. A mixture of 30% tungsten carbide, 30% molybdenum carbide, 20% vanadium carbide, 20% titanium carbide, etc. It is to be understood that these groupings and combinations are only given by way of example, and that this invention is by no means limited thereto.

This finely divided metal carbide powder, or combinations of metal carbide powders, is then placed in a carbide lined or stainless steel ball mill, and to this is added 6% by weight of finely divided pure cobalt metal powder, and the two are ball milled together for a sufficiently long time to uniformly distribute the cobalt throughout the mass. This first ball milling will take from 6 to 96 hours depending of course on the original fineness of the powders used. It is essential however to get a uniform distribution and a thorough commingling of all the ingredients. This I call refractory metal carbide mixture A.

I next prepare a bonding, densifying, and hardening mixture, which I call mixture B. This mixture consists of pure nickel, manganese, and copper powders, and beryllium in alloy form, either as nickel-beryllium alloy, or beryllium copper alloy. These powders are combined in a specific manner, and in a ratio in the order of 65% by weight of nickel, 25% by weight of manganese, and 10% by weight of copper. Although the beryllium may be added as a copper beryllium alloy replacing a portion of the copper, I find it more convenient to replace a portion of the nickel by a nickel beryllium alloy powder, containing 10% beryllium, so that the amount of beryllium in the alloy mixture B is not less than 0.25% and not more than 3% by weight. The presence of the small but effective amount of beryllium provides an alloy bonding material that can be heat treated to give a harder, tougher, and greater wear resistant body.

In preparing mixture B, I first weigh out the requisite amount of nickel powder 200 mesh and finer, and then add the required amount of the nickel beryllium alloy powder in finely divided form. The two are thoroughly mixed as by ball milling, until they are thoroughly commingled and uniformly distributed. This usually takes

from 1 to 4 hours. The manganese and the copper powder, both pure and in finely divided form, are then added in amounts specified below to bring the composition of this mixture to the required value.

|                     | Grams    |
|---------------------|----------|
| 1. Nickel powder    | 35-62.50 |
| 2. NiBe (10% alloy) | 30.0-2.5 |
| 3. Manganese powder | 25.0     |
| 4. Copper powder    | 10.0     |

All the powders are mixed and ball milled for a further period to get a thorough distribution of all the ingredients.

The proportions constituting alloy mixture B give a resultant alloy containing.

62.0-64.75% nickel  
3.0-2.5 Be  
25.0% Mn  
10.0% Cu

The final alloy mixture is then formed by thoroughly mixing from 90-60% of alloy mixture A and 10-40% of alloy mixture B. Here again it is important to get a thorough mixing to assure a uniform distribution of all the ingredients. The final mixture I call mixture C. The final mixing may be done dry in carbide lined or stainless steel ball mills using steel or carbide balls, or it may be done wet using carbontetrachloride or the like. If the final ball milling is done wet, care must be exercised to continue the mixing while the carbontetrachloride is driven off to prevent segregation of any of the ingredients. After thorough drying, mixture C can then be packed in air tight containers and is ready for use in making either diamond impregnated core bits, or, in combination with sintered hard metal carbide inserts, rotary type rock drilling bits, or in making any unit requiring a hard, tough abrasion resistant material.

Whether the alloy of this invention is to be used in making the diamond impregnated core bits or the rotary type rock drilling bits, the procedure except for modification of the carbon moulds and the manner of holding the abrasive grain, and/or the inserts in place, is the same. For the sake of simplicity I will describe a method of using the alloy of this invention in making a diamond impregnated core bit.

One form of apparatus as used in the hot pressing of the alloy of this invention, consists essentially of high frequency furnace with suitable controls for temperature, and a hydraulic press with suitable controls for pressure, having carbon or graphite moulds suitably machined to receive and hold the diamonds or cemented hard carbide inserts in place.

The graphite mould is circular in section and is suitably machined to give an annular recess and any desired bottom contour. In the bottom of this annular recess location points or grooves are drilled to receive and hold the diamonds in place. In operation the steps are as follows. The diamonds are carefully placed in the location grooves as described above. A weighed amount of alloy powder mixture C is then carefully placed in annular space, and uniformly distributed. A steel shank suitably machined, and having its bottom contour serrated, is then placed in the annular space on top of the alloy powder. The mould assembly is then placed in the high frequency furnace which is positioned on the bottom platen of a hydraulic press. Pressure is applied on top face of the shank until a value approximately

500 pounds per square inch on the pressing area of the alloy powder being pressed is reached. The high frequency current is turned on, quickly heating mould to the requisite temperature where it is held for a period of time sufficient to allow complete densification and alloying of all the ingredients. Temperature and time will depend on the particular composition used and the size and weight of the piece being pressed.

5 A 2" outside diameter x 1 1/4" inside diameter x 3/8" thick ring of the alloy of this invention was hot pressed and sintered and alloyed to a steel shank of the same outside and inside diameter dimensions in about 10 minutes. The high frequency furnace unit had a capacity of 30 kw. The initial cold pressure was approximately 500 pounds per square inch. The maximum temperature was 1250° C. and final pressure at maximum temperature was approximately 1000 pounds per square inch. As the temperature begins to rise it will be noted that the pressure drops due to partial sintering which begins to take place. Pressure however is maintained fairly constant throughout this pressing operation, and may even be increased to a higher value as the maximum temperature is approached. This pressure is maintained on the assembly until the pressed and sintered assembly has cooled down to approximately 800° C.

30 The pressure is then released and the assembly taken out of the furnace and allowed to cool quickly to approximate room temperature. The shank is then removed from the mould. It will be found that the diamonds protrude the predetermined amount, and are securely imbedded in the alloy material and that the steel shank has been thoroughly welded to the alloy forming a very strong tenacious bond.

40 It is obvious that furnaces other than high frequency furnaces may be used in practicing this invention. Any suitable furnace permitting quick heating of the mould and its contents and having the proper temperature controls will give equally good results.

45 The alloys of this invention containing 90% of mixture A and 10% of mixture B have a sintering temperature about 1350° C.-1500° C., whereas the alloys containing 60% mixture A and 40% mixture B have a sintering temperature of about 1100° C.-1200° C. Temperatures and pressures should be controlled within the limits specified to obtain an alloy of optimum properties.

50 Hardness of these alloys will vary depending naturally on the relative proportions of mixtures A and B used. For the 90% A-10% B combination the hardness is about 72-76 Rockwell C; for the 80% A-20% B, it is about 68-72; for the 70% A-30% B, it is about 60-64; and for the 60% A-40% B, it is about 56-60. All values are of hardness Rockwell C.

55 The combination that gave exceptionally good results were 70% mixture A and 30% mixture B; mixture A contributing 65.8% by weight of metal carbides, 4.2% by weight of cobalt and mixture B contributing 19.5% by weight of nickel plus beryllium combined, 7.5% by weight of manganese and 3% by weight of copper to the final alloy. The hardness of this pressed and sintered alloy was about 60-64 Rockwell C, and it was extremely tough, shock and abrasion resistant.

60 Coefficients of thermal expansion of this group of alloys are considerably higher than for the ordinary sintered carbide compositions. Values vary somewhat depending on composition. For the 90% A-10% B combination the coefficient is

approximately  $8.9 \times 10^{-6}$ , and for the 60% A-40% B it is  $12-13 \times 10^{-6}$ . For the 70% A-30% B combination it is  $12 \times 10^{-6}$ . Values given are in inches per inch per °C. and are approximate average values for the range 400-600° C. Because of these higher thermal expansion values, the alloy of this invention is particularly well adapted to be sintered and welded to the steel shanks ordinarily used in the mining and oil well industries. The use of this alloy as a crown material not only eliminates cracking and breakage due to extreme thermal strain but also eliminates a separate brazing operation of the crown to the shank.

It is to be understood that where reference is made to various metal carbides, that the respective saturated form of carbide is meant.

Having thus described my invention, what I claim is:

1. A pressed and sintered alloy of high strength and hardness, high thermal expansion and high abrasion and shock resistance comprising 90-60% by weight of a first separately prepared mixture and 10-40% by weight of a second separately prepared mixture in which said first mixture comprises 94% by weight of at least one metal carbide of the group consisting of tungsten, titanium, zirconium, vanadium, chromium, tantalum and molybdenum and 6% by weight of cobalt and said second mixture comprises 65% by weight of nickel and beryllium combined, 25% by weight of manganese and 10% by weight of copper in which the beryllium is not less than .25% nor more than 3.0% of the total of said second mixture.

2. A pressed and sintered alloy of high strength and hardness, high thermal expansion and high abrasion and shock resistance comprising 90-60% by weight of a first separately prepared mixture and 10-40% by weight of a second separately prepared mixture in which said first mixture comprises 94% by weight of tungsten carbide and 6% by weight of cobalt and said second mixture comprises 65% by weight of nickel and beryllium combined, 25% by weight of manganese and 10% by weight of copper in which the beryllium is not less than .25% nor more than 3.0% of the total of said second mixture.

3. A pressed and sintered alloy of high strength and hardness, high thermal expansion and high abrasion and shock resistance comprising 90-60% by weight of a first separately prepared mixture and 10-40% by weight of a second separately prepared mixture in which said first mixture comprises 79.9% by weight of tungsten carbide, 14.10% by weight of titanium carbide and 6% by weight of cobalt and said second mixture comprises 65% by weight of nickel and beryllium combined, 25% by weight of manganese and 10% by weight of copper in which the beryllium is not less than .25% nor more than 3.0% of the total of said second mixture.

4. A pressed and sintered alloy of high strength and hardness, high thermal expansion and high abrasion and shock resistance comprising 90-60% by weight of a first separately prepared mixture and 10-40% by weight of a second separately prepared mixture in which said first mixture comprises 47.0% by weight of tungsten carbide, 32.9% by weight of molybdenum carbide, 14.1% by weight of titanium carbide and 6% by weight of cobalt and said second mixture comprises 65% by weight of nickel and beryllium combined, 25% by weight of manganese and 10% by weight of copper in which the beryllium is not less than .25% nor more than 3.0% of the total of said second mixture.

5. A pressed and sintered alloy of high strength and hardness, high thermal expansion and high abrasion and shock resistance comprising 90-60% by weight of a first separately prepared mixture and 10-40% by weight of a second separately prepared mixture in which said first mixture comprises 28.2% by weight of tungsten carbide, 28.2% by weight of molybdenum carbide, 18.8% by weight of titanium carbide, 18.8% by weight of vanadium carbide and 6% by weight of cobalt and said second mixture comprises 65% by weight of nickel and beryllium combined, 25% by weight of manganese and 10% by weight of copper in which the beryllium is not less than .25% nor more than 3.0% of the total of said second mixture.

6. A pressed and sintered alloy of high strength and hardness, high thermal expansion and high abrasion and shock resistance consisting of 70% by weight of a first separately prepared mixture and 30% by weight of a second separately prepared mixture in which said first mixture comprises 94% by weight of tungsten carbide and 6% by weight of cobalt and said second mixture comprises 65% by weight of a nickel and beryllium alloy, 25% by weight of manganese and 10% by weight of copper in which said nickel beryllium alloy contains beryllium in an amount not less than .25% nor more than 3.0% of the total of said second mixture.

7. A pressed and sintered alloy of high strength and hardness, high thermal expansion and high abrasion and shock resistance consisting of 70% by weight of a first separately prepared mixture and 30% by weight of a second separately prepared mixture in which said first mixture comprises 79.9% by weight of tungsten carbide, 14.10% by weight of titanium carbide and 6% by weight of cobalt and said second mixture comprises 65% by weight of a nickel and beryllium alloy, 25% by weight of manganese and 10% by weight of copper in which said nickel beryllium alloy contains beryllium in an amount not less than .25% nor more than 3.0% of the total of said second mixture.

8. A pressed and sintered alloy of high strength and hardness, high thermal expansion and high abrasion and shock resistance consisting of 70% by weight of a first separately prepared mixture and 30% by weight of a second separately prepared mixture in which said first mixture comprises 47% by weight of tungsten carbide, 32.9% by weight of molybdenum carbide, 14.10% by weight of titanium carbide and 6% of cobalt and said second mixture comprises 65% by weight of a nickel and beryllium alloy, 25% by weight of manganese and 10% by weight of copper in which said nickel beryllium alloy contains beryllium in an amount not less than .25% nor more than 3.0% of the total of said second mixture.

9. A pressed and sintered alloy of high strength and hardness, high thermal expansion and high abrasion and shock resistance consisting of 70% by weight of a first separately prepared mixture and 30% by weight of a second separately prepared mixture in which said first mixture comprises 28.2% by weight of tungsten carbide, 28.2% by weight of molybdenum carbide, 18.8% by weight of titanium carbide, 18.8% by weight of vanadium carbide and 6% by weight of cobalt and said second mixture comprises 65% by weight of a nickel and beryllium alloy, 25% by weight of manganese and 10% by weight of copper in which said nickel beryllium alloy con-

tains beryllium in an amount not less than .25% nor more than 3.0% of the total of said second mixture.

JACOB KURTZ. 5

**REFERENCES CITED**

The following references are of record in the file of this patent:

**UNITED STATES PATENTS**

| Number    | Name          | Date          |
|-----------|---------------|---------------|
| 1,924,384 | Stoody        | Aug. 29, 1933 |
| 1,962,606 | Masing et al. | June 12, 1934 |
| 2,134,305 | Kieffer       | Oct. 25, 1938 |
| 2,160,670 | Oswald        | May 30, 1939  |
| 2,202,821 | Balke         | June 4, 1940  |
| 2,246,387 | Schwarzkopf   | June 17, 1941 |
| 2,349,052 | Ollier        | May 16, 1944  |
| 2,411,867 | Brenner       | Dec. 3, 1946  |
| 2,457,156 | Jones         | Dec. 28, 1948 |